

## UNITED STATES PATENT OFFICE

FRANCIS G. MOREHOUSE, OF GREENWICH, CONNECTICUT, ASSIGNOR TO RADIO CORPORATION OF AMERICA, A CORPORATION OF DELAWARE

## RECORDING PAPER

No Drawing.

Application filed December 18, 1929. Serial No. 415,141.

The present invention relates and has general application to systems for recording pictures and the like as received over wire or radio circuits at a receiving point which is located remotely from a transmitting station of any desired type. More particularly, the invention is directed to a suitable type of recording paper for recording the picture messages as they are received from the remotely located transmitting point.

Of course, by the term "pictures" as used throughout the specification, I mean any particular form of message which may be recorded to produce a representation which will affect the optical senses and convey information, and the term may include, views, photographs, financial statements, newspapers, magazine articles, advertisements, fashion plates, motion picture films, checks, documents, finger prints, and the like.

By my copending application, Serial No. 324,421, filed on December 7, 1928, jointly with Richard Howland Ranger, I have disclosed a system wherein it is possible to use heat for producing a record on a wax treated paper, and a system wherein the original application of heat by means of a process of selective absorption produces what has been termed a "latent image" on the paper. This "latent image" is, for example, a picture made up of a suitable aggregation of lines, dots, areas, etc., which are ink-absorptive against a background which is completely ink-repellent, or, in other words, the "latent image" portion of the record surface is absorptive to ink and the wax treated paper is repellent to ink.

As disclosed by the above named copending application, the "latent image" is produced by means of a jet of hot air projected against the paper, by a hot stylus made to touch the paper at different points thereon in accordance with received signals, or by any other heat producing means of sufficient heat intensity to melt the wax at points intended to represent the message. It is obvious that the more completely the local absorption of the wax coating into the paper support is attained, the more satisfactory will the finished record be, from the points of view of photo-

graphic contract and the general neatness and accuracy of recording. If the degree of wax-absorption is inadequate, it is found that the smallest dots and the finest lines of the "latent image", due to the heat application, are not faithfully brought out in good contrast by the inking process but tend to appear faint or are entirely absent from the finished record.

Therefore, as a primary object of the present invention, I have attempted to improve upon the process of recording by the use of a hot air jet, a hot stylus, or heat produced from a concentrated light source projected against the recording surface so as to melt the wax coating thereon and cause the same to be absorbed by the paper.

As a further purpose and object of my invention, I desire to produce a recording paper for use in the recording of pictures or the like which is more readily fusible than papers heretofore known and used, and which will require a lower degree of heat for producing any recording action, so that there may be a consequent longer life of the recording unit. I also desire to provide a recording sheet upon which greater recording speeds are possible, and a sheet which more closely approaches the speed of photographic recording sheets than has heretofore been known.

As a further object of my present invention, I desire to provide by means of the more complete selective absorption, a finished record which is a more faithful reproduction of the original, even to the finest dots and lines, than has heretofore been possible through the use of wax recording films or the like, and a record in which the degree of contrast between the finished picture and the background is materially improved.

Other objects and advantages, of course, will become apparent and readily suggest themselves to those skilled in the art to which the invention relates from a careful consideration of the following specification and claims forming a part of my disclosure.

According to the previous known methods for recording pictures or the like as a record on a heat sensitive paper of the wax type, it was customary to apply a thin film of wax in

liquid form (as, for example, from an aqueous colloidal emulsion or suspension) to one side of the paper sheet by surface dipping. After the wax coating thus placed upon one 5 surface of the paper was allowed to dry, it was desirable to polish the wax film with a soft hair brush, so as to smooth the surface and produce a polish thereon, and also to avoid some of the granulated effects due to 10 the unevenness of initial distribution of the wax film, which would be objectionable.

However, under such conditions, it was observed that upon the application of heat to the recording surface, the wax film thereon 15 was not melted at the low temperatures which were to be expected from considerations of the known melting point of the wax. Due to the fact that foreign substances of higher melting point were placed with the wax in 20 order to maintain the wax liquid in an emulsion state, the wax was not completely fused and therefore not absorbed by the paper stock sufficiently to permit sharp contrast when 25 ink was applied thereto at portions where the wax had been supposedly completely absorbed by the paper.

Therefore, according to my present invention, have sought to develop a method and means whereby the objectionable features of 30 this nature may be overcome, and as a means by which I accomplish the desired results, I have added what I have herein termed a "coagulant" as an additional coating on the paper, and have coated the paper in the following manner: to one surface of a sheet of absorbent paper, I have applied by surface dipping a "coagulant", to be hereinafter described, and have then permitted this coagulant to dry upon the sheet. After the coagulant 35 has been dried upon the sheet, I then apply a thin film of wax in the same manner as was previously done in the prior art, and which was disclosed in my copending application, reference to which has been made 40 above. I then allow this wax film to dry upon the paper, and I then polish the paper with a soft hair brush in the manner above described in connection with the paper having the coating only of wax.

50 Most of the commercial wax emulsions which are obtainable are apparently in the form of an aqueous suspension having a qualitative composition somewhat as follows: (a) wax (such as paraffin); (b) soaps (as emulsifying agents); (c) preservatives, stabilizers, etc.; (d) an aqueous vehicle. The addition of the coagulant to the coating upon the recording surface is intended to function or serve to increase the fusibility of the wax film. 55 Such coagulants as may be used may be either of the organic or the inorganic type. Where coagulants of the organic type are used, they should be such organic compounds as dissolve in water to form an acid solution, and 60 may consist, for example, of tartaric acid,

acetic acid, phthalic acid, oxalic acid, benzoic acid, citric acid, and other organic compounds of like nature. Where it is desired to use inorganic substances as coagulants, these inorganic compounds should be such 70 that they dissolve in water to form an acid solution, and may consist, for example, of nickel sulphate, copper sulphate, ferric chloride, strontium chloride, cadmium sulphate, manganese nitrate, lead nitrate, lead acetate, aluminum sulphate, chromium sulphate, aluminum nitrate, and other inorganic compounds of like nature.

While experimentation has indicated what is apparently the true chemical theory of 80 operation of the coagulant with respect to the wax emulsion so as to produce reactions such that make the entire composition more readily fusible and permit a lower degree of heat to be used in recording, and a consequent 85 longer life of recording unit, I wish it to be distinctly understood that any theory which I may herein express is not to be regarded as limiting my invention, but is disclosed simply for the purpose of more clearly explaining the nature thereof in the manner in 90 which I at present understand it. This theory may be expressed somewhat as follows: As the wax emulsion is applied to the paper coated with the coagulant as above stated, 95 the process of application to the paper partially dissolves the coagulant, which is believed to interact with the wax emulsion, and the following altered composition apparently results by virtue of the acidity of the dissolved coagulant: First, the wax (such as the paraffin) apparently remains unchanged; second, the free fatty acids corresponding to the soaps used as emulsifying agents are produced; third, the preservatives stabilizers, etc. remain unchanged; and fourth, the aqueous vehicles remains unchanged, but, of course, dries out, as stated above, to form the dry wax film on the paper. It is thus observed that the soaps are the only ingredients that undergo any change due to the presence of the coagulant, and experimentation indicates that the film resulting from the application to the paper of the mixture of the wax, the free fatty acids, the preservatives, 110 stabilizers, and the aqueous vehicle, is more readily fusible than the film resulting from the mixture of wax, soaps, preservatives, stabilizers and the aqueous vehicle, since the soaps tend to prevent the deposited film from 115 melting to a mobile, freely absorbable liquid of low viscosity. The free fatty acids, however, do not offer any such prevention, but on the contrary seem to permit the deposited film to melt sharply under heat to a very 120 free-flowing liquid, which is readily and completely absorbed by the paper support, to expose an area of excellent ink-absorbing qualities.

Thus, the "latent image" formed from the 130

application of heat represents a more complete attainment of the condition of selective absorption than has heretofore been obtainable, and, after inking, the record exhibits improved faithfulness of reproduction and better contrast.

Many modifications and changes in the present invention will at once suggest themselves and become apparent to those skilled in the art to which the invention relates, and while I have hereinabove illustrated by way of example several of the many substances which I may use as coagulants, I believe that I am entitled to use any and all of such substances as fall fairly within the spirit and scope of the invention as defined by the hereinafter appended claims.

Having now described my invention, what I claim and desired to secure by Letters Patent is the following:

- 20 1. A heat sensitive recording sheet provided with a coagulant and a wax film on the surface thereof.
- 25 2. A heat sensitive recording sheet having a coagulant coating on the surface thereof, and a waxy emulsion superposed upon the coagulant.
- 30 3. A heat sensitive recording sheet having an inorganic coagulant coating the surface thereof, and a waxy emulsion superposed upon the coagulant.
- 35 4. The process of preparing papers for heat sensitive recording which consists in coating the paper stock with a coagulant, and, after drying, again coating the paper provided with a coagulant on the surface thereof with a waxy heat sensitive emulsion.
- 40 5. The process of preparing a paper stock for heat sensitive recording which consists in coating one surface of the paper stock with a coagulant, drying the coated paper, coating the dried paper stock provided with the coagulant with a waxy emulsion, and in again drying the entire sheet.
- 45 6. A heat sensitive recording sheet having an organic coagulant coating the surface thereof, and a waxy emulsion superposed upon the said coagulant.

FRANCIS G. MOREHOUSE:

50

55

60

65